

# United States Patent

[11] 3,620,852

[72] Inventors **Robert B. Herchenroeder**  
Kokomo, Ind.;  
**Joe G. Y. Chow, Northport; Albert H.**  
**Fleitman, Smithtown, N.Y.**  
[21] Appl. No. **15,237**  
[22] Filed **Feb. 27, 1970**  
[45] Patented **Nov. 16, 1971**  
[73] Assignee **The United States of America as**  
**represented by the United States Atomic**  
**Energy Commission**

[54] **PROCESS FOR PRODUCING COBALT ALLOYS**  
2 Claims, No Drawings

[52] U.S. Cl. .... **148/2,**  
75/171, 148/11.5  
[51] Int. Cl. .... **C22f 1/10,**  
C22c 19/00  
[50] Field of Search ..... **148/2, 3,**  
**11.5, 12; 75/122, 177**

[56] **References Cited**  
UNITED STATES PATENTS  
2,564,498 8/1951 Nisbet ..... 75/170 A  
2,920,956 1/1960 Nisbet et al. ..... 75/171 K  
3,356,542 12/1967 Smith ..... 75/171  
3,366,478 1/1968 Wheaton ..... 75/171  
3,432,294 3/1969 Wheaton ..... 75/171  
*Primary Examiner—Charles N. Lovell*  
*Attorney—Roland A. Anderson*

**ABSTRACT:** A process for producing oxygen-free cobalt based alloys having improved stability in high temperature irradiated sodium environments wherein cobalt is alloyed with chromium, tungsten, iron, carbon, nickel, molybdenum and titanium and thereafter the alloy is cold reduced 50 percent and heat annealed until it has a grain size of less than 10 microns.

## PROCESS FOR PRODUCING COBALT ALLOYS

## PRIOR ART

The nuclear power industry is planning on constructing breeder-type reactors using molten sodium as a coolant. The contemplated use of molten sodium poses many safety and material problems. It requires containment materials such as pipes for transporting the sodium through the reactor.

The piping in such reactors must be capable of containing sodium, at high temperature in heavy fields of nuclear radiation. Conventional alloys have so far proven unequal to the task for a variety of reasons. Thus the art is seeking a metal alloy which can withstand the rigors of such an environment.

## SUMMARY OF INVENTION

A method of producing cobalt-based alloys, said alloys having stability in high temperature, radiation and sodium environment comprising charging a furnace with from 71.02 to 42.0 weight percent cobalt, based on the total weight of the alloy, from 24.0 to 19.03 weight percent chromium, based on the total weight of the alloy, from 21.84 to 4.92 weight percent nickel, based on the total weight of the alloy, from 16.0 to 4.50 weight percent of at least one member of the group consisting molybdenum and tungsten based on the total weight of the alloy, from 8.30 to 0.18 weight percent iron based on the total weight of the alloy, up to about 1.0 weight percent titanium based on the total weight of the alloy, about 0.03 weight percent carbon based on the total weight of the alloy, about 0.03 weight percent carbon based on the total weight of the alloy; heating the charge to a temperature ranging from about 2,500° F. to about 2,700° F. for a period ranging from about 15 to 20 minutes while maintaining the charge under a vacuum of less than three microns a mercury; adding an oxygen getter to remove any oxygen from the heated charge; and removing the oxygenated getter from the charge; cooling the heated charge to its freeze point and adding from 5.26 to 0.09 weight percent titanium based upon the total weight of the alloy; back-pressuring the chamber over the charge with an inert gas, e.g., argon; heating the charge containing the titanium under an atmosphere of inert gas to a temperature above 2,500° F. until a uniform melt is obtained; adding a sulfur getter to fix any sulfur contained in the charge, pouring the charge into a mold and cooling the cooling the poured charge until it is a solid billet; working the billet until it has a grain size of less than 10 microns by conventional means, e.g., reducing the billet thickness by 50 percent while maintaining the billet at a temperature below 2,100° F. and thereafter heating the reduced billet at a temperature of about 1,600° F. for about 16 hours.

## DETAILED DESCRIPTION OF THE INVENTION

The process of our invention can be carried out using conventional alloying techniques and equipment. Care must be taken to eliminate oxygen as an impurity from the alloy. Thus, the alloy is heated under a vacuum of three microns or less until a homogeneous melt is obtained. Oxygen-getters are added to the melt to remove any oxygen impurities from the melt.

Our invention can utilize conventional oxygen-getters such as, but not limited to, aluminum, zirconium and magnesium and titanium. In the preferred embodiment of our invention, we employ aluminum as the oxygen-getter because it has a low vapor pressure, reacts quickly with the oxygen in the system and the aluminum oxide thus formed floats on top of the melt and adheres to the crucible and is thus readily removed with any other slag contained on the melt.

The titanium in our alloy is added after oxygen impurities have been removed from the melt due to the high degree of reactivity between titanium and oxygen and the fact that only a small weight percent of titanium is desired in our alloying process.

After the melt is degassed, the vacuum chamber over the melt is backfilled with a partial pressure of an inert gas to

assist in the retention of the high-vapor pressure sulfur getter, e.g., magnesium or mixtures of nickel and magnesium which is added to fix (tie up sulfur as a stable compound and prevent hot shortness) residual sulfur and to prevent undesirable melt-crucible reactions during the casting of the alloy.

After the alloys have been poured and cooled into a solid billet, we reduce (roll) the billet until its thickness has been reduced by about 50 percent. This reduction can be done at temperatures under 2,100° F. preferably is done at room temperature. Conventional milling equipment can be utilized to obtain the reduction.

The final annealing at a low temperature, e.g., 1,600° F. for a time period sufficient to cause recrystallization and secondary precipitation of particles is important as this annealing, together with the prior reduction produces a structure having a final grain size of less than 10 microns.

In selecting materials for the alloy, care should be taken to select materials which are substantially free of silicon, boron, and other impurities. Such impurities have a deleterious effect on the alloy performance in the higher temperature radiation sodium environment in which it is planned to employ the alloy.

Table I show several alloy samples which were made up in accordance with the practice of this invention. The figures given in this table are weight percentages based upon the total weight of the alloy.

TABLE I

|    |       | A     | B     | C     | D |
|----|-------|-------|-------|-------|---|
| Cr | 21.37 | 21.21 | 21.37 | 21.26 |   |
| W  | 5.15  | 4.72  | 5.17  | 5.15  |   |
| Fe | 8.20  | 8.20  | 8.30  | 8.30  |   |
| C  | 0.03  | 0.025 | 0.025 | 0.028 |   |
| Ni | 10.08 | 10.06 | 10.09 | 10.10 |   |
| Mo | 4.87  | 5.03  | 5.03  | 5.09  |   |
| Ti | 0.09  | 0.21  | 0.46  | 0.64  |   |
| Co | Bal.  | Bal.  | Bal.  | Bal.  |   |

These sample alloys were prepared as follows:

Raw materials -cobalt granules, electrolytic nickel and low-impurity iron, vacuum grade chromium, melting grade tungsten, molybdenum pellets, sponge titanium, high-carbon chromium and zirconium sponge.

Melting Sequence -A vacuum induction furnace was charged with cobalt, chromium, nickel, tungsten, iron, molybdenum, and high-carbon chrome containing carbon equal to about 0.025 weight percent of the total charge. The vacuum chamber was then evacuated and the temperature slowly raised to 2,500° F. as measured by an optical pyrometer (because of the necessity of sighting through an extra glass in the vacuum shell, the optical pyrometer readings are approximately 150° F. less than the actual temperature. Therefore, a recorded optical pyrometer measurement of 2,500° F. would mean that the actual temperature of the melt was approximately 2,650° F.).

After the cessation of the carbon boil and accompanying degassing, the temperature was reduced to the liquidus point of the melt and late additions of aluminum titanium, and powdered graphite were added and the temperature was again raised to 2,500° F. as measured by the optical pyrometer. At this point, the chamber was backfilled with argon to approximately one-half atmosphere pressure and a quantity of magnesium, in the form of nickel-magnesiu, was plunged into the bath to fix the residual sulfur content. The melt was then cast into one nominally 15-pound round tapered ingot, one nominally 20-pound ingot and samples for chemistry and other analysis. The results of the chemistry analysis are shown in table I.

The ingots were the hot reduced (about 2,100° F.) in thickness to within about 30 percent of their final diameter and were coldswaged to their final size in the shape of rods and the billets were then heat annealed at a temperature of about 1,600° F. for 16 hours.

A microscopic examination of these rods showed that they had a grain size structure of less than three microns.

The annealed billets were then subject to irradiation at a fluency of  $1.3 \times 10^{20}$  with the E > 0.82 million electron volts. The flux during irradiation was about  $10^{13}$  neutrons per square centimeter per second.

Table II, shown below, shows the results of yield tensile and elongation tests on the four different alloys shown in table I after they had been irradiated.

A comparison of tables II and III discloses the beneficial results obtained when our novel alloying process is utilized to prepare alloys for use in high temperature irradiated environments.

We claim:

1. A method of producing cobalt based alloys, said alloys having stability in high temperature, radiation and sodium environment comprising;

a. charging a furnace with from 71.02 to 42.0 weight per-

TABLE II.—EFFECTS OF IRRADIATION ON COBALT BASE ALLOY\* COLD WORKED AND RECRYSTALLIZED

| Alloy Sample No. | Irrad. fluence         | Test temp., °C. | Yield strength, p.s.i. | Tensile strength, p.s.i. | Total elongation, percent |
|------------------|------------------------|-----------------|------------------------|--------------------------|---------------------------|
| A-----           | 0                      | 750             | 31,200                 | 33,000                   | 57                        |
|                  | 0                      | 800             | 17,500                 | 19,000                   | 87                        |
|                  | $**1.3 \times 10^{20}$ | 650             | 80,000                 | 95,000                   | 29                        |
|                  | $**1.3 \times 10^{20}$ | 750             | 32,400                 | 39,800                   | 24                        |
|                  | $**1.3 \times 10^{20}$ | 800             | 24,400                 | 26,200                   | 67                        |
| B-----           | 0                      | 25              | 116,000                | 179,000                  | 28                        |
|                  | 0                      | 650             | 74,600                 | 82,400                   | 45                        |
|                  | 0                      | 750             | 31,700                 | 33,400                   | 52                        |
|                  | 0                      | 800             | 18,500                 | 19,800                   | 63                        |
|                  | $1.3 \times 10^{20}$   | 650             | 81,200                 | 97,560                   | 20                        |
|                  | $1.3 \times 10^{20}$   | 750             | 41,500                 | 42,600                   | 22                        |
| C-----           | 0                      | 25              | 117,000                | 178,000                  | 15                        |
|                  | 0                      | 650             | 72,300                 | 84,500                   | 34                        |
|                  | 0                      | 750             | 32,900                 | 35,000                   | 47                        |
|                  | $1.3 \times 10^{20}$   | 650             | 20,700                 | 22,300                   | 71                        |
|                  | $1.3 \times 10^{20}$   | 750             | 80,500                 | 94,800                   | 23.5                      |
|                  | $1.3 \times 10^{20}$   | 750             | 41,500                 | 44,100                   | 28                        |
| D-----           | 0                      | 25              | 126,000                | 160,500                  | 4-                        |
|                  | 0                      | 650             | 78,800                 | 92,500                   | 5-                        |
|                  | 0                      | 750             | 29,300                 | 32,100                   | 6-                        |
|                  | 0                      | 800             | 16,700                 | 19,000                   | 7-                        |
|                  | $1.3 \times 10^{20}$   | 650             | 79,700                 | 94,800                   | 2-                        |
|                  | $1.3 \times 10^{20}$   | 750             | 40,300                 | 42,700                   | 3-                        |
|                  | $1.3 \times 10^{20}$   | 800             | 26,400                 | 28,000                   | 7-                        |

\*\*E 0.82 Mev.

NOTE: All specimens tested at a strain rate of 0.2% per min.

Table III, shown below, shows the results of yield, tensile and elongation tests on cobalt alloys and on iron base alloy which were prepared by conventional techniques.

Table III

Comparison of Properties of Iron and Cobalt Base Alloys  
(All specimens irradiated at less than 100° C. to  $1.3 \times 10^{20}$  E 0.82 MeV)

Not Cold Worked and Recrystallized

| Alloy                                      | Test Temp. °C. | Yield Strength, p.s.i. | Tensile Strength, p.s.i. | Total Elonga-tion % |
|--------------------------------------------|----------------|------------------------|--------------------------|---------------------|
| Cobalt Base (10Ni-20Cr-15W)                | 25             | 139,000                | 142,000                  | 15 X                |
|                                            | 650            | 45,000                 | 70,000                   | 17                  |
|                                            | 750            | 35,000                 | 38,000                   | 9.2                 |
|                                            | 800            | 39,200                 | 41,500                   | 2.3                 |
| Cobalt Base UMCO 15 (28Cr-20Fe-2Cb)        | 25             | 120,000                | 146,000                  | 26                  |
|                                            | 650            | 46,400                 | 68,600                   | 9                   |
|                                            | 750            | 38,700                 | 46,600                   | 7.5                 |
|                                            | 800            | 34,200                 | 39,600                   | 6.5                 |
| Conventional 25* Iron Base Stainless Steel |                |                        |                          |                     |
|                                            | 600            | 81,500                 | 105,000                  | 58                  |
|                                            | 650            | 26,000                 | 40,600                   | 14                  |
|                                            | 650            | 19,200                 | 29,800                   | 7.5                 |
|                                            | 650            | 24,800                 | 31,700                   | 14                  |
|                                            | 700            | 23,000                 | 23,900                   | 10                  |
|                                            | 750            | 15,800                 | 18,100                   | 13                  |
|                                            | 800            | 10,500                 | 11,700                   | 6                   |

cent cobalt, based upon the total weight of the alloy; from 24.0 to 19.03 weight percent chromium, based on the total weight of the alloy; from 21.84 to 4.92 weight percent nickel based upon the total weight of the alloy; consisting of molybdenum and tungsten, based upon the total weight of the alloy; from 8.3 to 0.18 weight percent titanium, based on the total weight of the alloy; and about 0.03 weight percent carbon, based upon the total weight of the alloy;

b. heating the charge to a temperature ranging from about 2,500° F. to about 2,700° F. for a period ranging from about 15 to about 20 minutes while maintaining the charge under a vacuum of less than 3 microns of mercury;

c. adding an oxygen getter to the charge to remove any oxygen from the heated charge;

d. cooling the heated charge to its freeze point and adding from 5.26 to 0.09 weight percent titanium based upon the total weight of the alloy;

e. backpressuring the chamber over the charge with an inert gas;

f. heating the charge to a temperature above 2,500° F. until a uniform melt is obtained and adding a sulfur getter in amounts sufficient to fix the residual sulfur;

g. pouring the charge into a mold and cooling the poured charge until it is a solid billet;

h. working the solid billet until it has a grain size of less than 10 microns by reducing the billet thickness about 50 percent while maintaining the billet at a temperature below 2,100° F. and thereafter heating the reduced billet at a temperature of about 1,600° F. for about 16 hours.

2. A method in accordance with claim 1 wherein the solid billet is worked until it has a grain size of less than 3 microns.

\*Strain rate 2 percent per minute, all other specimens strained at 0.2 percent per minute. Ps